# EUROPEAN PATENT SPECIFICATION

(11) **EP 1 669 475 B1**
(45) Date of publication and mention of the grant of the patent: **28.10.2009**
(21) Application number: 05026729.3
(22) Date of filing: 07.12.2005
(51) Int. Cl.: C23C 22/34, B05D 7/14

(54) **Pretreatment method and powder coating step for coating surface of metal for vehicle chassis**
Vorbehandlung für eine Metalloberfläche und Pulverbeschichtungsschritt für ein Fahrgestell
Pretraitement d'une surface métallique et étappe de revêtment en poudre pour un châssis3

(30) Priority: 08.12.2004 JP 2004355455
(43) Date of publication of application: 14.06.2006
(73) Proprietor: Nippon Paint Co., Ltd., Osaka-shi Osaka 531-8511 (JP); Hino Motors, Ltd., Hino-shi, Tokyo 191-8660 (JP)
(72) Inventor: Makino, Kazuhiro c/o NIPPON PAINT CO.,LTD., Tokyo 140 8675 (JP); Hashimoto, Aki c/o NIPPON PAINT CO.,LTD., Tokyo 140 8675 (JP); Futsuhara, Masanobu c/o NIPPON PAINT CO.,LTD., Tokyo 140 8675 (JP); Shimakura, Toshiaki c/o NIPPON PAINT CO.,LTD., Tokyo 140 8675 (JP); Kobayashi, Takehiko, Hino-shi, Tokyo 191-8660 (JP); Murakami, Eikou, Hino-shi, Tokyo 191-8660 (JP)
(74) Representative: Brehm, Hans-Peter

(56) References cited:
- EP-A- 1 433 877
- EP-A- 1 455 002

## Description

### TECHNICAL FIELD

The present invention relates to a method of applying a powder coating onto a hot rolled and shot blasted steel plate to be used as a vehicle chassis component,
wherein this method comprises
- a pre-treatment step (1) of pretreating the hot rolled and shot blasted steel plate with a chemical conversion treatment solution in order to form a chemical conversion coat; and
- a coating step (2) of powder coating the pretreated steel plate as pretreated by the pre-treatment step (1).

### BACKGROUND ART

Vehicle chassises are generally constructed of a steel lumber such as a hot rolled steel lumber, or of a steel lumber from which a modified layer such as mill scale or the like is removed by shot blasting or the like. A typical coating method is powder coating which is performed subsequently to the chemical conversion treatment of said steel lumbers by means of zinc phosphate treating agents. Known pretreatment methods for coating the surface of metal for vehicle chassis by such treating agents are described in the documents Japanese Kokai Publication Hei-10-204649 and 2002-220678.

Japanese Kokai Publication Hei-10-204649 discloses an aqueous zinc phosphate solution which may form a coat having good adhesion of coating and providing good corrosion resistance even when omitting a specific surface conditioning step. This chemical conversion coat is obtained by means of a chemical conversion treatment solution containing specific components such as phosphate ions, zinc ions, a hydroxylamine source and the like in specific amounts.

Japanese Kokai Publication 2002-220678 discloses a method of treating hot rolled steel sheets or steel lumber with a zinc phosphate treating agent containing specific components such as phosphate ions, zinc ions, manganese ions, nickel ions and the like in specific amounts to provide a coat having good corrosion resistance.

However, the use of zinc phosphate treating agents causes environment protection problems, especially due to bad economy and bad workability of the waste water treatment caused by the high metal ion concentration, and by the high acid concentration and by the handling of an extremely reactive treating agent. Further, the metal surface treatment with the zinc phosphate treating agents causes the formation of water-insoluble salts which are deposited as a precipitate. Such a precipitate is generally referred to as a sludge, and removal and dumping of said sludges provides additional costs. Since phosphate ions may burden the environment by eutrophication, a treatment of liquid wastes is required, and it is more preferred to avoid the formation of those liquid wastes. Further, the metal surface treatment with zinc phosphate containing treating agents requires a surface conditioning step, and this surface conditioning step makes the overall complete process time consuming.

Other metal surface treating agents, than the zinc phosphate treating agents are known in the metal coating art. For example, the documents Japanese Kokai Publications 2001-316845 and 2001-516810 describe metal surface treating agents comprising zirconium compounds. Such a zirconium compound containing metal surface treating agent shows in so far an excellent property compared with respect to the zinc phosphate containing chemical conversion treating agents as described above, because the use of the zirconium compound containing metal surface treating agent does not cause the formation of sludge.

But, when the surface of metal for vehicle chassis is treated with the above mentioned zirconium compound containing metal surface treating agent, it was difficult to obtain chemical conversion coats having adequate adhesion of the chemical conversion coat and to provide an adequate post-coating corrosion resistance.

The document EP 1 455 022 A1 is related to a pre-treatment method for coating, comprising the following features:
- treating a substance to be treated with a chemical conversion coating agent to form a chemical conversion coat;
- wherein the chemical conversion coating agent comprises at least one kind selected from the group consisting of zirconium, titanium and hafnium and fluorine;
- the chemical conversion coat has a fluorine concentration of 10% or less on the atom ratio basis; and
- at least a part of the substance to be treated is an iron material.

The chemical conversion coating agent may additionally contain at least one further component selected from a group consisting of magnesium, calcium, a silicon-containing compound, zinc and copper. The silicon containing compound is not particularly limited, and examples thereof may include silica, water-soluble silicate compounds, ester of silicic acid, alkyl silicates, silane coupling agents and the like. The silane coupling agent is not particularly limited and, for example, an amino group-containing silane coupling agent is suitably used. The amino group-containing silane coupling agent is a compound having at least an amino group and having a siloxane linkage in a molecule, and examples thereof may include publicly known silane coupling agents such as N-2(aminoethyl)3-aminopropylmethyldimethoxy-silane, N-2(aminoethyl)3-aminopropyltrimethoxy-silane, N-2(aminoethyl)3-aminopropyltriethoxy-silane, 3-aminopropyltrimethoxy-silane, 3-aminopropyltriethoxy-silane, 3-triethoxysilyl-N-(1,3-dimethyl-butylidene)propylamine, N-phenyl-3-aminopropyltrimethoxy-silane and N,N-bis[3-(trimethoxysilyl)propyl]ethylendediamine. The silane coupling agent may include hydrolysates thereof, polymers thereof, and the like.

Said document describes along with Example 13 thereof the preparation of a test sheet, wherein a commercially available cold-rolled steel sheet is treated with a chemical conversion coating agent containing 100 ppm zirconium and 200 ppm hydrolysate of 3-aminopropyl trimethoxy-silane.

The selection of the iron material to be treated is not particularly limited, and examples thereof may include a cold-rolled steel sheet, a hot-rolled steel sheet and the like.

The fore-mentioned pre-treatment method may be followed by a coating step wherein a coating is applied onto the pretreated article. Examples thereof may include coatings using a cationic electrodeposition coating composition, an organic solvent coating composition, a water-borne coating composition, a powder coating composition and so on. The document contains not less than 20 inventive Examples, and each one of the Examples 1 to 20 demonstrate only the coating obtained by the cationic electrodeposition coating method.

Further, the document EP 1 433 877 A1 describes a pre-treatment method for coating. The content of the document EP 1 433 877 A1 is very close and similar to the content of the fore-mentioned document EP 1 455 002 A1.

### SUMMARY OF THE PRESENT INVENTION

In view of the above-described state of the art, it is the object of the present invention to provide for a method of applying a powder coating onto a hot rolled and shot blasted steel plate to be used as a vehicle chassis component,
wherein this method comprises
- a pre-treatment step (1) of pretreating the hot rolled and shot blasted steel plate with a chemical conversion treatment solution in order to form a chemical conversion coat; and
- a coating step (2) of powder coating the pretreated steel plate as pretreated by the pre-treatment step (1);
a chemical conversion treatment solution and a pre-treatment step which enable
- to obtain a chemical conversion coat having an adequate adhesion and an adequate corrosion resistance;
- without the necessity of using phosphates:
- to maintain the formation of sludge extremely small; and
- to facilitate the treatment of the waste water accrued during said pre-treatment step.

Accordingly, the present invention provides
a method
of applying a powder coating onto a hot rolled and shot blasted steel plate to be used as a vehicle chassis component,
wherein this method comprises
- a pre-treatment step (1) of pretreating the hot rolled and shot blasted steel plate with a chemical conversion treatment solution in order to form a chemical conversion coat; and
- a coating step (2) of powder coating the pretreated steel plate as pretreated by the pre-treatment step (1);
**wherein**
said chemical conversion treatment solution comprises
- zirconium in an amount of 50 to 500 ppm referred to the metal element equivalent basis;
- at least one silane compound selected from a group consisting of γ-aminopropyltriethoxysilane, hydrolysates of γ-aminopropyltriethoxysilane, γ-aminopropyltrimethoxysilane and hydrolysates of γ-aminopropyltrimethoxysilane; and
- a pH of from 2 to 6; and
this pre-treatment step (1) is performed at a temperature of from 30 °C to 60 °C during a treatment period of from 30 to 300 seconds.

According to a preferred embodiment of the method according to the present invention the pretreated steel plate as pretreated by the pre-treatment step (1) is rinsed with water and is tried or air blowed before effecting the coating step (2) of powder coating.

According to a further preferred embodiment of the method according to the present invention, the hot rolled and shot blasted steel plate is subjected to an alkaline degreasing step and rinsing with water before performing the pre-treatment step (1) , but omitting any further surface conditioning step prior to said pre-treatment step (1).

Along with the method according to the present invention, it is possible to form and obtain a chemical conversion coat having good adhesion and good corrosion resistance without the necessity of performing a surface conditioning step prior to said pre-treatment step (1).

According to a further preferred embodiment of the method according to the present invention the chemical conversion treatment solution contains y-aminopropyl-triethoxysilane, hydrolysates of y-aminopropyltriethoxysilane, y-aminopropyl-trimethoxysilane or hydrolysates of y-aminopropyltrimethoxysilane in an amount of from 50 to 50.0 ppm.

According to a still further embodiment of the method according to the present invention the chemical conversion treatment solution further contains 50 to 500 ppm of magnesium ions and/or 50 to 1000 ppm of zinc ions.

### DETAILED DESCRIPTION OF THE PRESENT INVENTION

Hereinafter, the present invention is described in more detail.

When performing the method according to the present invention and a piece of hot rolled and shot blasted steel plate is contacted with a weakly acidic aqueous solution of fluorozirconic acid, Fe²⁺ ions are eluted due to an etching reaction at an anode reaction site portion, and the pH at an interface increases due to a reduction reaction of hydrogen at a cathode reaction site to precipitate a hydroxide of zirconium. At the anode reaction site, the eluted Fe²⁺ ions catch fluoride ions to form a complex fluoride ion of ZrF₆⁻ , and thereby said hydroxide of zirconium is precipitated similarly. The coat of the precipitated zirconium hydroxide is a closely packed amorphous coat and this coat can inhibit the permeation of water or chlorine ions to the underlying metal surface; thus, the metal is corrosion protected. A silanol group of the selected aminosilane reacts through dehydration condensation with a hydroxyl group of said zirconium hydroxide precipitated on the surface of metal to form a metalloxan bond. It is considered that an amino group of said aminosilane is oriented to the direction of the coating film and forms a strong chemical bond by reacting with a functional group of the coating film, and thereby the adhesion to the coating film is enhanced. The thus formed chemical conversion coat may present a performance which is equal to or higher than the performance of the conventional zinc phosphate coat, both with respect to the corrosion resistance and the adhesion of the coat.

The method of applying a powder coating onto a hot rolled and shot blasted steel plate according to the present invention includes the pre-treatment of a surface of a steel lumber modified by a surface oxidation step (not rolling), wherein a modified surface layer such as mill scale or the like is removed by shot blasting or the like.

The here used chemical conversion treatment solution contains zirconium in an amount of 50 to 500 ppm on the metal element equivalent basis. When the zirconium content is less than 50 ppm, then the formation of the chemical conversion coat is insufficient and the corrosion resistance of said chemical conversion coat is also insufficient. When the zirconium content amounts more than 500 ppm, then an additional effect is not be expected and a higher zirconium content is unfavorable due to economic reasons. Even more preferred is a chemical conversion treatment solution comprising a zirconium content of from 75 ppm to 300 ppm.

The selection of a resource for providing said zirconium content within the chemical conversion treatment solution is not particularly limited; for example the following zirconium containing compounds may be used:
alkali metal fluorozirconates such as K₂ZrF₆ and the like;
fluorozirconates such as (NH₄)₂ZrF₆ and the like;
soluble fluorozirconates such as fluorozirconic acid, such as H₂ZrF₆, and the like;
zirconium fluoride; and
zirconium oxide.

Here, fluorozirconicacid (H₂ZrF₆) andammoniumfluorozirconates [(NH₄)₂ZrF₆] are preferred, because they do no influence the chemical conversion properties.

The method according to the present invention uses a chemical conversion treatment solution which contains at least one silane compound selected from γ-aminopropyltriethoxysilanes, hydrolysates thereof, γ-aminopropyltrimethoxysilanes and hydrolysates thereof. These amino silane compounds contain at least one amino group in their molecule and comprise a siloxane bond. These compounds act on both, the chemical conversion coat and on the subsequently applied coating film; thereby, the adhesion between the chemical conversion coat and the coating film is improved.

The hydrolysates, of these amino silane compounds maybe obtained by hydrolysis of γ-aminopropyltriethoxysilane or of γ-aminopropyltrimethoxysilane, and by hydrolysis of condensates formed by condensation reaction of these substances.

Preferably, this chemical conversion treatment solution comprisesy-aminopropyltriethoxysilane, hydrolysates thereof, γ-aminopropyltrimethoxysilane and hydrolysates thereof in an amount of from 50 ppm to 500 ppm. If this amino silane compound content is less than 50 ppm, then the formation of a coat may be insufficient and the corrosion resistance of the thus formed chemical conversion coat may also be insufficient. If this amino silane compound content is higher than 500 ppm, then an additional effect is not be expected, and a higher amino silane compound content may be unfavorable due to economic reasons. Even more preferred is a chemical conversion treatment solution containing said amino silane compounds in a content of from 75 ppm to 300 ppm.

A commercially available source for the above-stated γ-aminopropyltriethoxysilane is KBE-903 (trade name) produced by Shin-Etsu Chemical Co., Ltd. or Sila-Ace S-330 (trade name) produced by CHISSO CORPORATION.

A commercially available source for the above γ-aminopropyltrimethoxysilane is KBM-903 (trade name) produced by Shin-Etsu Chemical Co., Ltd. or Sila-Ace S-360 (trade name) produced by CHISSO CORPORATION.

Preferably, the method according to the present invention uses a chemical conversion treatment solution which contains additionally magnesium ions. This content of magnesium ions improves the adhesion and the corrosion resistance of the chemical conversion coat. Preferably, this magnesium ions content has a lower limit of 50 ppm and an upper limit of 500 ppm. If this magnesium content is less than 50 ppm, then the formation of a chemical conversion coat may be insufficient and the corrosion resistance thereof may also be insufficient. If this magnesium content is higher than 500 ppm, then an additional effect is not be expected, and a higher magnesium content is unfavorable due to economic reasons. Even more preferred is a chemical conversion treatment solution having a magnesium ions content of from 75 ppm to 400 ppm.

These magnesium ions maybe provided by adding magnesium nitrate, magnesium sulfate, magnesium carbonate and the like.

Preferably, the method according to the present invention uses a chemical conversion treatment solution containing additionally zinc ions. This content of zinc ions improves the adhesion and the corrosion resistance of the chemical conversion coat. Preferably, this zinc ions content has a lower limit of 50 ppm and an upper limit of 1000 ppm. If this zinc content is less than 50 ppm, then the formation of a chemical conversion coat may be insufficient and the corrosion resistance thereof may also be insufficient. If this zinc content is higher than 1000 ppm, then an additional effect is not be expected, and a higher zinc content may be unfavorable due to economic reasons. Even more preferred is a chemical conversion treatment solution having a content of zinc ions of from 100 ppm to 750 ppm.

These zinc ions, may be provided by adding zinc nitrate, zinc sulfate, zinc carbonate and the like.

The method according to the present invention uses a chemical conversion treatment solution having a pH within a range of from 2 (lower limit) to 6 (upper limit). If the pH is lower than 2, then the etching becomes excessive, and a formation of the chemical conversion coat cannot be adequately achieved. If the pH is higher than 6, then the etching becomes insufficient, and a good chemical conversion coat is not obtained. Even more preferred is a ph within a range of from 2.5 to 5.0.

In order to adjust the pH of the chemical conversion treatment solution, acidic compounds such as nitric acid, sulfuric acid and the like, or basic compounds such as sodium hydroxide, potassium hydroxide, ammonia and the like may be added.

Preferably, the method according to the present invention uses a chemical conversion treatment solution which does not contain phosphate ions in an substantial amount. Here "a not substantial amount" means that phosphate ions are not contained to such an extent that they act as a component in the chemical conversion treatment solution. Thus, the formation of sludge such as iron phosphate sludge, zinc phosphate sludge and the like, as produced when using a zinc phosphate containing treatment agent, can be avoided.

In addition to the above-stated components, the chemical conversion treatment solution as used with the method according to the present invention may additionally contain arbitrary components, as required. For example, arbitrary components such as silica and the like may be mentioned. By adding such an arbitrary component to the solution, the post-coating corrosion resistance may be improved.

When performing the method according to the present invention, the kind and method of contacting the hot rolled and shot blasted steel plate with the chemical conversion treatment solution is not particularly limited, and usual treatment conditions may be used, for example, an immersion step, a spraying step, a roll coating step and the like, may be mentioned.

According to the method of the present invention, the chemical conversion treatment is carried out at a temperature in the range of from 30°C to 60 °C during a treatment period of from 30 seconds to 300 seconds. If the treatment temperature is lower than 30 °C, then the chemical reactivity is low and an adequate chemical conversion coat is not formed, further the corrosion resistance of this coat may be poor. If this treatment temperature is higher than 60°C, then an additional effect is not be expected; the higher treatment temperature is unfavorable due to economic reasons. Even more preferred is a treatment temperature in the range of from 35°C to 50 °C. If the treatment duration is less than 30 seconds, then an adequate chemical conversion coat cannot be obtained and the corrosion resistance thereof may be poor. If this treatment duration is longer than 300 seconds, then an additional effect is not to be expected; the longer treatment duration may be unfavorable due to economic reasons. Even more preferred is a treatment duration period ranging of from 45 seconds to 240 seconds.

When performing the method according to the present invention, an amount of a chemical conversion coat deposited on the treated steel plate is preferably ranging of from 5 mg/m² to 300 mg/m² in terms of the total metal content contained in the used chemical conversion treatment solution. If this amount of chemical conversion coat is less than 5 mg/m², then the obtained chemical conversion coat is not uniform. If this amount of chemical conversion coat is higher than 300 mg/m², then an additional effect is not to be obtained; this higher amount is unfavorable due to economic reasons. Even more preferred is an amount of chemical conversion coat deposited on the treated steel plate in a range of from 10 mg/m² to 200 mg/m².

As a matter of facts, a hot rolled and shot blasted steel plate to be treated according to the method of the present invention may often contain adhering oil typically to be removed by an alkaline degreasing treatment and followed by subsequent rinsing with water. Typically, this alkaline degreasing treatment comprises a step immersing the steel plate for several minutes into an alkaline degreasing cleaning solution and/or a phosphorus- and nitrogen-free degreasing cleaning solution having a temperature of from 30 °C to 55°C. This alkaline degreasing treatment is followed by a post-degreasing rinsing step, which is typically performed by spraying a large amount of rinsing water one or more times onto the degreased steel plate in order to rinse and remove the above-stated degreasing agent(s).

Further, it is known in the art to perform a pre-degreasing treatment before performing the fore-mentioned alkaline degreasing treatment.

This kind of alkaline degreasing treatment - may be with preceding pre-degreasing treatment - may also be performed with a hot rolled and shot blasted steel plate, before treating said steel plate along with the method according to the present invention.

If the conventional treatment of a steel plate witch phosphate solution is intended, then a surface conditioning step is required subsequent to the alkaline degreasing step and the water rinsing step (s).

Contrarily thereto, even if a conventional alkaline degreasing treatment - even including a preceding pre-degreasing step- is performed before treating the thus degreased and rinsed steel plate along with the method according to the present invention, then a conventional surface conditioning step is not required. Thus, a preferred embodiment of the present invention comprises a mode of treatment steps wherein the hot rolled and shot blasted steel plate is subjected to an alkaline degreasing step and rinsing with water before performing the pre-treatment step (1), according to the method of the present invention, but omitting any further surface conditioning step prior to said pre-treatment step (1).

Accordingly, even if the conventional alkaline degreasing treatment of a surface of metal article for vehicle chassis is performed before subsequently performing the method according to the present invention, does not require the above-mentioned surface conditioning step to be performed after alkaline degreasing and rinsing treatment with water. A chemical conversion coat having good adhesion to the coating applied by subsequent powder coating step and a good corrosion resistance may be obtained by a multiple consecutive step method comprising lesser steps.

The present invention provides
a method
of applying a powder coating onto a hot rolled and shot blasted steel plate to be used as a vehicle chassis component,
wherein this method comprises
- a pre-treatment step (1) of pretreating the hot rolled and shot blasted steel plate with a chemical conversion treatment solution in order to form a chemical conversion coat; and
- a coating step (2) of powder coating the pretreated steel plate as pretreated by the pre-treatment step (1).

Preferably, further steps are provided subsequent to said pre-treatment step (1) and prior to said coating step (2). Along with said further steps the pretreated steel plate as pretreated by the pre-treatment step (1) is rinsed with water and is dryed or air blowed before effecting the coating step (2) of powder coating.

If said rinsing with water step subsequently to the pre-treatment step (1) is insufficient, then the subsequently applied layer obtained by powder coating shows a bad film appearance. Therefore the pre-treated steel plate is rinsed with water two times or more subsequent to the pre-treatment step (1). Further, it is appropriate to perform the final rinsing step with pure water. The temperature of said pure water is preferably a temperature in the range of from 20 ° C to 80 ° C.

All said steps from alkali degreasing to rinsing with pure water subsequent to the pre-treatment step (1) may be performed by either spray water rinsing or immersion water rinsing.
Therefore, these steps may be carried out by means of already existing equipments.

Preferably, subsequent to said water rinsing steps subsequent to the pre-treatment step (1), a drying step or an air blowing step is performed. Drying or air blowing is preferably carried out at a temperature ranging of from room temperature to 120 ° C. A drying time is preferably 5 seconds to 10 minutes.

The subsequent powder-coating a step (2) may be carried out by conventional powder coating methods, for example, by methods comprising: applying a powder coating composition to the plate surface to be coated by electrostatic spray coating, by fluidized bed dip coating or the like; and heating the powder coating composition on the surface of the coated plate to become melted and cured; and cooling the coated plate.

The selection of a suited powder coating composition is not particularly limited; for example, a composition containing an epoxy resin, an acrylic resin, a polyester resin or the like as a main binder and further containing a curing agent such as polyhydric carboxylic acid, blocked isocyanate or the like may be mentioned.

### BEST MODES FOR CARRYING OUT THE INVENTION

Hereinafter, the present invention will be described in more detail by means of Examples, but the present invention is not limited to these Examples. Further, "part(s)" or "%" refers to "part (s) by weight" or "% by weight" , respectively.

### Preparation of the chemical conversion treatment solution to be used in Example 1:

H₂ZrF₆ (200 ppm as Zr) was dissolved in water; to this solution were added: Mg (NO₃)₂ (200 ppm as Mg) and Zn (NO₃)₂ (500 ppm as Zn), and finally a required amount of γ-APS (γ-APS stands for γ-aminopropyltriethoxysilane); the thus obtained solution was stirred thoroughly, and finally adjusted to a pH of 4.0 by means of ammonia water.

### Example 1:

A shot blasted hot rolled steel plate (70 mm x 150 mm x 5 mm, obtained from Nippon Testpanel Co., Ltd.) was cleaned at 42°C for 2 minutes with an alkaline degreasing agent (SURFCLEANER EC92, produced by NIPPON PAINT Co., Ltd.), rinsed with water, and treated at 40°C for 90 seconds with the fore-mentioned chemical conversion treatment solution. Then, the pre-treated plate was rinsed with water and further rinsed with pure water of 60 °C; thereafter an air blowing step was performed to dry the plate. Then, a powder coating composition (Powdax P200 black, a polyester powder coating composition produced by NIPPON PAINT Co., Ltd.) was applied on the plate by electrostatic spraying. The applied powder composition was baked by maintaining for 20 minutes at 160 °C so as to obtain a film thickness of 50 mm on the plate.

### Examples 2 to 6 and Comparative Examples 1 to 3:

The chemical conversion treatment of the steel plates was performed in the same manner as described in Example 1 except for changing the concentrations of the components of the chemical conversion treatment solution and the temperature and the treatment time of the pre-treatment step to values as shown in Table 1. Then, the obtained pre-treated steel plates were rinsed with water, dried, and powder-coated.

### Comparative Example 4:

The same kind of steel plate as used in Example 1 was cleaned with an alkaline degreasing agent, rinsed with water, surface-treated by immersion in a surface conditioner (SURFFINE 5N-8R, produced by NIPPON PAINT Co., Ltd.) at room temperature for 30 seconds, and then immersed in a conventional zinc phosphate treating agent (SURFDINE SD5350, produced by NIPPON PAINT Co., Ltd.) at 35°C for 2 minutes. Then, this steel plate was rinsed with water, dried, and powder-coated in the same manner as described in Example 1.

### Evaluation by means of Salt spray test (SST):

The surface of the powder coated steel plate was cross-cutted (10 cm × 10 cm) by means of a cutter. Thereafter, the cross-cutted plate was treated at 35°C for 360 hours by spraying a 5% aqueous solution of NaCl. Then, the width of rust formed on both sides of the cut portion was measured and was evaluated according to the following criteria.
O: the width of rust is less than 5 mm;
×: the width of rust is 5 mm or more

The results of evaluation are shown in the following Table 1.

**Tabelle 1:**

| | | **Zr concentration (ppm)** | **Mg concentration (ppm)** | **Zn concentration (ppm)** | **γ-APS (ppm)** | **Temperature (°C)** | **Time (sec)** | **SST performance** |
|---|---|---|---|---|---|---|---|---|
| Examples according to the present invention | 1 | 200 | 200 | 500 | 200 | 40 | 90 | ○ |
| | 2 | 60 | 400 | 250 | 60 | 45 | 90 | ○ |
| | 3 | 450 | 60 | 900 | 450 | 35 | 40 | ○ |
| | 4 | 100 | 100 | 200 | 100 | 55 | 35 | ○ |
| | 5 | 150 | 100 | 60 | 100 | 35 | 280 | ○ |
| | 6 | 200 | 200 | 400 | 200 | 40 | 60 | ○ |
| Comparative Examples | 1 | 30 | 30 | 30 | 30 | 40 | 120 | × |
| | 2 | 60 | 30 | 30 | 40 | 40 | 25 | × |
| | 3 | 100 | 100 | 100 | 100 | 25 | 60 | × |
| | 4 | treated with zinc phosphate | | | | | | ○ |

As shown with Table 1, the steel plates pre-treated according to the method of the present invention show the good corrosion resistances. Comparative Examples 1 and 2 use a lesser content of γ-APS; comparative Example 3 uses a lower temperature for the pre-treatment step. The steel plates pre-treated according to Comparative Examples 1 to 3 show the poor corrosion resistance. The corrosion resistance of the steel plates obtained according to inventive Examples 1 to 6 is equal or higher than the corrosion resistance of the steel plate obtained according to Comparative Example 4 treated with conventional zinc phosphate conversion agent without performing a surface conditioning step.

### INDUSTRIAL APPLICABILITY

The method according to present invention may be suitably used as the pretreatment method for coating the surface of hot rolled and shot blasted steel plates for vehicle chassis. This method facilitates waste water treatment and provides a chemical conversion coat having good adhesion and good corrosion resistance without performing the surface conditioning step.

## Claims

1. A method
of applying a powder coating onto a hot rolled and shot blasted steel plate to be used as a vehicle chassis component,
wherein this method comprises
- a pre-treatment step (1) of pretreating the hot rolled and shot blasted steel plate with a chemical conversion treatment solution in order to form a chemical conversion coat; and
- a coating step (2) of powder coating the pretreated steel plate as pretreated by the pre-treatment step (1);
**wherein**
said chemical conversion treatment solution comprises
- zirconium in an amount of 50 to 500 ppm referred to the metal element equivalent basis;
- at least one silane compound selected from a group consisting of γ-aminopropyltriethoxysilane, hydrolysates of γ-aminopropyltriethoxysilane, γ-aminopropyltrimethoxysilane and hydrolysates of γ-aminopropyl-trimethoxysilane; and
- a pH of from 2 to 6; and
this pre-treatment step (1) is performed at a temperature of from 30 to 60°C during a treatment period of from 30 to 300 seconds.

2. The method according to claim 1
**wherein**
the pretreated steel plate as pretreated by the pre-treatment step (1) is rinsed with water and is dryed or air blowed before effecting the coating step (2) of powder coating.

3. The method according to Claim 1 or 2,
**wherein**
the hot rolled and shot blasted steel plate is subjected to an alkaline degreasing step and rinsing with water before performing the pre-treatment step (1), but omitting any further surface conditioning step prior to said pre-treatment step (1).

4. The method according to anyone of Claims 1 to 3,
**wherein**
the chemical conversion treatment solution contains γ-aminopropyl-triethoxysilane, hydrolysates of γ-aminopropyltriethoxysilane, γ-aminopropyl-trimethoxysilane or hydrolysates of γ-aminopropyltrimethoxysilane in an amount of from 50 to 500 ppm.

5. The method according to anyone of Claims 1 to 4,
**wherein**
the chemical conversion treatment solution further contains 50 to 500 ppm of magnesium ions and/or 50 to 1000 ppm of zinc ions.

## Patentansprüche

1. Verfahren
zum Aufbringen einer Pulverbeschichtung auf warmgewalztem und strahlentzundertem Stahlblech,
das als Fahrzeugchassiskomponente eingesetzt werden soll,
wobei dieses Verfahren aufweist:
- einen Vorbehandlungsschritt (1) zur Vorbehandlung des warmgewalzten und strahlentzunderten Stahlbleches mit einer chemischen Umwandlungslösung, um einen Überzug aus chemischer Umwandlungslösung zu erzeugen; und
- einen Beschichtungsschritt (2), um das gemäß vorstehendem Vorbehandlungsschritt (1) vorbehandelte Stahlblech mit einer Pulverbeschichtung zu versehen,
**dadurch gekennzeichnet, dass**
diese chemische Umwandlungslösung aufweist:
- Zirconium in einem Anteil von 50 bis 500 ppm bezogen auf die Aequivalentbasis an metallischen Elementen;
- wenigstens eine Silanverbindung, ausgewählt aus einer Gruppe, die umfasst: γ-Aminopropyl-triethoxy-silan, Hydrolysate von γ-Aminopropyl-triethoxy-silan, γ-Aminopropyl-trimethoxy-silan und Hydrolysate von γ-Aminopropyl-trimethoxy-silan;
- sowie einen pH-Wert von 2 bis 6; und
dieser Vorbehandlungsschritt (1) bei einer Temperatur von 30 bis 60 °C während einer Behandlungsdauer von 30 bis 300 Sekunden ausgeführt wird.

2. Verfahren nach Anspruch 1,
**dadurch gekennzeichnet, dass**
das, gemäß diesem Vorbehandlungsschritt (1) vorbehandelte Stahlblech mit Wasser gespült und getrocknet oder mit einem Luftstrahl behandelt wird, bevor der Beschichtungsschritt (2) der Pulverbeschichtung durchgeführt wird.

3. Verfahren nach Anspruch 1 oder 2,
**dadurch gekennzeichnet, dass**
das am warmgewalzten und strahlentzunderten Stahlblech eine Entfettungsbehandlung mit einem alkalischen Medium durchgeführt wird und daraufhin mit Wasser gespült wird, bevor der Vorbehandlungsschritt (1) ausgeführt wird;
wobei jedoch vor diesem Vorbehandlungsschritt (1) keine weitere Oberflächenkonditionierungsmaßnahme durchgeführt wird.

4. Verfahren nach einem der Ansprüche 1 bis 3,
**dadurch gekennzeichnet, dass**
die chemische Umwandlungslösung γ-Aminopropyl-triethoxy-silan, Hydrolysate von γ-Aminopropyl-triethoxy-silan, γ-Aminopropyl-trimethoxy-silan und Hydrolysate von γ-Aminopropyl-trimethoxy-silan in einem Anteil von 50 bis 500 ppm enthält.

5. Verfahren nach einem der Ansprüche 1 bis 4,
**dadurch gekennzeichnet, dass**
die chemische Umwandlungslösung zusätzlich 50 bis 500 ppm Magnesiumionen und/oder 50 bis 1.000 ppm Zinkionen enthält.

## Revendications

1. Un procédé
d'application d'un revêtement en poudre sur
de la tôle d'acier laminée à chaud et grenaillée
pour l'utilisation comme composant de châssis de véhicule,
ce procédé comprenant
- une étape de prétraitement (1) pour le prétraitement de la tôle d'acier laminée à chaud et grenaillée avec une solution de conversion chimique pour produire une couche de conversion chimique ; et
- une étape de revêtement (2) pour appliquer un revêtement en poudre sur la tôle d'acier prétraitée conformément à l'étape de prétraitement (1),
**caractérisé en ce que**
la solution de conversion chimique présente :
- du zirconium de l'ordre de 50 à 500 ppm par rapport à la base d'équivalent éléments métalliques ; et
- au moins un composé de silane choisi d'un groupe comprenant :
du γ-aminopropyl triéthoxy silane, des hydrolysates d'y-aminopropyl triéthoxy-silane, γ-aminopropyl triméthoxy silane et des hydrolysates de γ-aminopropyl triméthoxy silane ;
- une valeur pH entre 2 et 6 ; et que
cette étape de prétraitement (1) est réalisée à une température entre 30 et 60°C pendant une durée de traitement entre 30 et 300 secondes.

2. Le procédé conformément à la revendication 1,
**caractérisé en ce que** :
la tôle d'acier prétraitée conformément à l'étape de prétraitement (1) est rincée à l'eau et séchée ou traitée au jet d'air avant d'être soumise à l'étape de revêtement (2) par application du revêtement en poudre.

3. Le procédé conformément à la revendication 1 ou 2,
**caractérisé en ce que** :
la tôle d'acier laminée à chaud et grenaillée est soumise à un traitement de dégraissage avec un agent alcalin et qu'elle est rincée ensuite avant d'être soumise à l'étape (1) ;
sans qu'il y ait cependant avant l'étape (1) une autre étape de conditionnement de la surface.

4. Le procédé conformément à une des revendication 1 à 3,
**caractérisé en ce que** :
la solution de conversion chimique contient du γ-aminopropyl triéthoxy silane, des hydrolysates de γ-aminopropyl triéthoxy-silane, γ-aminopropyl triméthoxy silane et des hydrolysates de γ-aminopropyl triméthoxy silane de l'ordre de 50 à 500 ppm.

5. Le procédé conformément à une des revendication 1 à 4,
**caractérisé en ce que** :
la solution de conversion chimique contient en plus 50 à 500 ppm d'ions de magnésium et/ou 50 à 1.000 ppm d'ions de zinc.
